

July 20, 1965

S. V. R. MASTRANGELO

3,196,090

PROCESS FOR PRODUCING FLUORINE AND SODIUM-LEAD ALLOY

Filed March 12, 1962

2 Sheets-Sheet 1

**FIG. I**



BY *Edwin C. Woodhouse*

ATTORNEY

July 20, 1965

S. V. R. MASTRANGELO

3,196,090

PROCESS FOR PRODUCING FLUORINE AND SODIUM-LEAD ALLOY

Filed March 12, 1962

2 Sheets-Sheet 2

**FIG. 2**



**FIG. 3**



3,196,090  
**PROCESS FOR PRODUCING FLUORINE AND  
SODIUM-LEAD ALLOY**  
Sebastian V. R. Mastrangelo, Wilmington, Del., assignor  
to E. I. du Pont de Nemours and Company, Wilming-  
ton, Del., a corporation of Delaware  
Filed Mar. 12, 1962, Ser. No. 178,938  
10 Claims. (Cl. 204—60)

This invention relates to a process for the production of elemental fluorine and sodium-lead alloy by the electrolysis of molten sodium fluoroborate in the presence of a molten lead cathode.

Fluorine is a valuable commodity which has a wide variety of important uses, such as the preparation of inorganic fluorine compounds and organic fluorine-containing compounds. At the present time, elemental fluorine is prepared commercially by the electrolysis of hydrogen fluoride or of sodium bifluoride. These processes produce hydrogen as the cathode product which, while useful, is more readily and more economically produced from petroleum refining and the electrolysis of acidified water or brine. It would be desirable to obtain a commercially more valuable product as the cathode product, such as sodium-lead alloy which is useful for a wide variety of purposes and particularly for reaction with alkyl chlorides to form tetraalkyllead compounds that are widely used as antiknock agents in hydrocarbon fuels for internal combustion engines. Sodium bifluoride cannot be used for the electrolytic production of fluorine and sodium-lead alloy because it produces hydrogen at the cathode and furthermore it decomposes appreciably at the melting point of lead so that it cannot be used with a molten lead cathode.

It has been proposed to electrolyze various metal fluorides to produce fluorine and other products, sometimes at temperatures below 300° C. but usually at temperatures of 600° C. and above. However, at 600° C. and above, elemental fluorine is highly corrosive and rapidly reacts with carbon to produce fluorinated organic compounds. Accordingly, it is impractical to use carbon anodes at such high temperatures for the production of elemental fluorine because of the production of fluorinated organic products with corresponding large decreases in the yield of elemental fluorine, and rapid consumption of the carbon anode.

It is an object of this invention to provide a new and improved electrolytic process for preparing elemental fluorine. Another object is to provide a process for preparing elemental fluorine which simultaneously produces sodium-lead alloy as the cathode product. A further object is to provide a process of the above character which produces an anode product which can be readily purified to produce substantially pure elemental fluorine and to reform the electrolyte. Still another object is to advance the art.

The above and other objects may be accomplished in accordance with this invention wherein elemental fluorine and sodium-lead alloy are produced simultaneously by the process which comprises electrolyzing an electrolyte consisting essentially of molten anhydrous sodium fluoroborate in an inert atmosphere at a temperature of from 385° C. to 500° C. in an electrolytic cell having an anode composed of a member of the group consisting of graphite, microcrystalline carbon, explosively compacted graphite, silicon carbide, and gold, and a cathode consisting essentially of molten lead at substantially the same temperature as the electrolyte, employing an electric current of from 2 to about 25 volts to provide a current

density of from 2 to 50 amperes per square decimeter (amps./dm.<sup>2</sup>) of anode surface area, recovering a sodium-lead alloy as the cathode product and a gaseous mixture of elemental fluorine and boron trifluoride as the anode product, and separating the elemental fluorine from the boron trifluoride.

A further important feature of this invention comprises the steps of separating the elemental fluorine from the boron trifluoride by passing the gaseous mixture 10 through sodium fluoride at a temperature of from about 200° C. to about 500° C. whereby the boron trifluoride reacts with the sodium fluoride to reform sodium fluoroborate and recycling the reformed sodium fluoroborate to the electrolytic cell.

15 The process of the invention is more economical than those processes which produce hydrogen as the cathode product, particularly because of the greater value of the sodium-lead alloy produced. Under the conditions employed, the sodium fluoroborate and the anode products, elemental fluorine and boron trifluoride, do not react with carbon to a significant extent, whereby a carbon anode can be employed without consumption of the anode and the production of significant amounts of fluorine-containing organic compounds. The gaseous 20 mixture of elemental fluorine and boron trifluoride can be readily separated by reaction of the boron trifluoride with sodium fluoride to give essentially pure elemental fluorine and to reform sodium fluoroborate from the boron trifluoride, which contributes materially to the 25 economics of the process and is particularly advantageous for continuous operation of the process.

The electrolyte should consist essentially of molten anhydrous sodium fluoroborate. Small amounts of sodium fluoride up to about 2% by weight can be tolerated, 30 but larger amounts have the tendency to raise the melting point of the electrolyte to above the temperatures required for the present process. Also, the sodium fluoroborate should be free of chlorine-containing materials so as to avoid contamination of the anode product with 35 chlorine. Water must be completely absent because it tends to hydrolyze the sodium fluoroborate to boric oxide and because water reacts with fluorine to form oxygen difluoride which is highly explosive.

Sodium fluoroborate has a melting point of about 383° 40 C. to 385° C. The electrolysis should be carried out at a temperature of from 385° C. to about 500° C. and preferably from about 440° C. to about 480° C. At temperatures above 500° C., sodium fluoroborate tends to decompose to sodium fluoride and boron trifluoride. Also, 45 at temperatures materially above 500° C., sodium fluoroborate and the anode products become highly corrosive and materially more reactive and tend to react with carbon and, where a carbon anode is employed, produces fluorine-containing carbon compounds resulting in loss in 50 the production of elemental fluorine and consumption of the carbon anode.

In the process of this invention, the cathode consists 55 essentially of a pool of molten lead. The molten lead should be substantially pure, as significant amounts of other metals cannot be permitted in the sodium-lead alloy, particularly when such alloy is to be used for making tetraalkyllead compounds.

The anode should consist of a conductor composed 60 of graphite, microcrystalline carbon, explosively compacted graphite, silicon carbide or gold. In most cases, graphite, particularly explosively compacted graphite, is preferred. Explosively compacted graphite and its preparation are disclosed in Belgian Patent No. 598,362, 65 granted January 13, 1961, to E. I. du Pont de Nemours and Company as assignee of Chrisp, Dieter, Jr., and 70

Jenkins. In some cases, such as in the use of a skull furnace, it will generally be preferred to employ a gold anode. In the gold anode, the gold may be plated as an external coating on another material such as graphite, copper or the like.

The reactions involved in the process are represented by the following equations wherein e represents an electron, (g) means gas, (s) means solid, and (liq.) means liquid:

Cathode reaction:



Anode reaction, carbon anode:



$\text{BF}_3$  recovery:



Anode reaction, gold anode:



Unlike the other anodes which merely act as conductors of electricity, part of the gold electrode takes part in the reaction, forming auric fluoride which decomposes to gold and fluorine at the reaction temperature. More specifically,  $\text{BF}_4^-$  reacts at the gold anode to form  $\text{BF}_3$  and  $\text{F}_2$ . The fluorine immediately reacts with the gold to form  $\text{AuF}_3$  (auric fluoride). The auric fluoride apparently does not adhere to the gold electrode but floats away on top of the molten electrolyte. At temperatures greater than  $385^\circ \text{ C.}$  auric fluoride is not stable and decomposes to gold and fluorine. The resulting gold is in a very finely divided colloidal state which floats on the molten electrolyte, possibly due to surface tension effects of the melt. After a short time, the gold film on top of the molten electrolyte is continuous and forms part of the anode. The film then is continuously being converted to auric fluoride and back to gold. Colloidal gold, in spite of the high density of gold, is known to remain suspended in water indefinitely, so it is not surprising that it floats on the molten electrolyte.

In the operation of the process, there should be employed a direct electric current of from 2 to about 25 volts to provide a current density of from 2 to 50 amperes per square decimeter (amps./dm.<sup>2</sup>) of anode surface area, usually 2 to about 25 amps./dm.<sup>2</sup>, preferably from 2 to about 7 volts and a current density of from 2 to about 20 amps./dm.<sup>2</sup> and most preferably between 2 and 3 volts and current densities of from 2 to about 4.7 amps./dm.<sup>2</sup>. The current densities and voltages are interrelated. The voltage required to obtain any current density is primarily a function of the anode material used. Current densities lower than about 2 amps./dm.<sup>2</sup> cause a very slow production rate, although they are operable. At current densities above 25 amps./dm.<sup>2</sup>, polarization of the electrodes tends to produce undesirable effects and, at current densities materially above 50 amps./dm.<sup>2</sup>, erosion of the anode and severe polarization of the electrodes occur which require higher voltages to obtain the same current densities or render the system inoperative.

The anode products, elemental fluorine and boron trifluoride, have very low boiling points whereby it is difficult to separate them by fractional distillation or fractional condensation. However, in accordance with the present invention, they are readily separated by passing the gaseous mixture over anhydrous sodium fluoride, usually preheated to about  $200^\circ \text{ C.}$  to about  $500^\circ \text{ C.}$  Under such circumstances, the boron trifluoride reacts to reform sodium fluoroborate, the elemental fluorine

does not react with the sodium fluoride and hence passes on to be collected and stored for use. Usually, an excess of sodium fluoride is employed to insure the complete removal of the boron trifluoride from the gaseous mixture. The resulting sodium fluoroborate therefore usually contains some sodium fluoride and it is then treated with further amounts of boron trifluoride at about  $400^\circ \text{ C.}$ , employing sufficient boron trifluoride to substantially completely convert the sodium fluoride to sodium fluoroborate which can then be recycled to the electrolytic cell.

Suitable forms of electrolytic cells for practicing the process of this invention are illustrated in the accompanying diagrammatic drawings in which FIG. 1 is a view in vertical cross section of one form of cell; FIG. 15 2 is a horizontal cross section taken on line 2-2 of FIG. 1; and FIG. 3 is a view in vertical cross section of second form of cell.

Referring particularly to FIGS. 1 and 2, the cell is of a general H-form having two vertical tubular legs 10 and 12 connected by a horizontal tubular cross member 14 at approximately  $\frac{1}{3}$  the height of the legs, to provide a passage for the flow of liquid between said legs 10 and 12. Said members 10, 12 and 14 are made of a heat resistant metal such as nickel, Inconel or the like, and are provided with inner linings 16 of a refractory material such as solid sodium fluoride, solid calcium fluoride, or a solid fused mixture of NaF and CaF<sub>2</sub>. The lower  $\frac{3}{4}$  (approximate) of the cell is provided with a heating jacket 18 which as shown is in the form of insulated electric heating elements. Cooling coils 20 of tubing for the circulation of a cooling fluid, e.g., water, surround the upper portions of the legs 10 and 12 to maintain the upper portions of the cell at a temperature such that the metal will not be seriously attacked by the gaseous products.

The leg 10 has a cap 22 having a charging port 24, a port cover 26, and gaskets 23 and 25. A discharge port 28 for discharging sodium-lead alloy is provided in the bottom of leg 10 and is closed by a suitable valve (not shown). An electrical connector 30 projects into the leg 10 near the bottom thereof and into the molten lead or molten sodium-lead alloy 32 which is maintained in leg 10 below the level of the passage formed by the cross member 14 and forms the cathode of the cell.

The leg 12 is closed at the bottom and may terminate at the level of the bottom of the cross member 14, if desired. The leg 12 is provided with a cover 34 which has a gas discharge port 36. The cover 34 also supports a carbon anode 38 fitted through a compression seal 40 which preferably is made of polytetrafluoroethylene or like inert material and which is held in place by a cap 42. Gaskets are also provided at 35 and 41. The lower end of the anode 38 dips into the electrolyte 44 above the level of the passage provided by the cross member 14. Means for introducing an inert gas, such as nitrogen, may be provided in cover 34, if desired.

In operation, sodium fluoroborate is added via charging port 24 and melted by means of heaters 18, the amount being sufficient to fill the cell for approximately  $\frac{2}{3}$  its height, i.e., at about the level indicated at 44, and so as to extend above the lower end of the anode. Lead is then added, via port 24, to the desired level indicated at 32, i.e., below the level of cross member 14. Direct current is applied across the anode and the cathode. Sodium forms at the lead cathode 32 and dissolves therein to form sodium-lead alloy. Fluorine and boron trifluoride form at the anode 38 and pass out of the reactor via port 36. The fluorine and boron trifluoride are separated by passing the mixture over anhydrous sodium fluoride. The boron trifluoride reacts with the sodium fluoride to reform sodium fluoroborate and the nonreacting elemental fluorine passes on to be collected and stored for use. The sodium fluoroborate recovered is returned periodically to the reactor via port 24. Periodically, part

of the liquid cathode 32 is withdrawn as sodium-lead alloy, and fresh lead is added via port 24. It is best not to allow the concentration of sodium in the cathode 32 to exceed about 5% to avoid reaction of sodium with sodium fluoroborate to form elemental boron which is undesired.

FIG. 3 shows an electrolytic cell of the so-called "skull-furnace" type in which the molten electrolyte and the molten lead cathode are contained in a shell formed of solid electrolyte. This type of cell is particularly useful with a gold anode, but may also be used with a carbon anode. This cell comprises a cylindrical vessel 46 and a cover 48, both made of a heat resistant metal such as nickel, Inconel, or the like. The cover is provided with a charging port 50 closed by a cover 52, and with a gas discharge port 54. Also, the cover 48 carries at its center an anode 56 fitted through a compression seal 58 which preferably is made of polytetrafluoroethylene or like inert material and which is held in place by a cap 60. Gaskets are also provided as in the structure of FIG. 1. A vertical pipe 62, made of a metal which is a good conductor of electricity and is heat resistant, passes up through the bottom of the vessel 46, offset from but near the center of said bottom, and has its open end terminating approximately  $\frac{1}{3}$  the height of the vessel 46. Said pipe 62 is provided with a valve 64 and is separated from the bottom of the vessel by an electrical insulator 66. Also, said pipe 62 is connected to the source of electric current so as to form an electrical connector for the molten lead cathode 68. Means for introducing an inert gas, such as nitrogen, may be provided in the cover 48, if desired.

The cell of FIG. 3 is operated by filling the vessel 46 to near the top with solid sodium fluoroborate and passing current between the anode 56 and the pipe 62, generating sufficient heat to melt part of the solid sodium fluoroborate to form a pool 70 of liquid sodium fluoroborate in the center of the upper portion of the solid sodium fluoroborate 72, said pool extending from below the upper end of pipe 62 to considerably above said end. With the current off, lead is quickly added through port 50. The lead melts and sinks to the bottom of the pool

The cell shown in FIG. 3 has the advantage that it permits the use of a gold anode. In the cell of FIG. 3, the gold which forms a film on top of the molten electrolyte 70, cannot come into contact with the metal walls of the vessel 46. Otherwise, the whole vessel 46 would become part of the anode and the cell would cease to operate.

The hazards of handling elemental fluorine are well known. In particular, materials which react with fluorine rapidly should be scrupulously excluded from the reaction system. These particularly include organic materials such as oils, greases, waxes, pipe dopes and the like, water, oxygen, reactive metals, and the like. Therefore, the process is carried out under an inert atmosphere in the cell. Any air, which may be present in the cell after charging the cell with the electrolyte and the lead cathode, will be small in amount and is quickly swept out with the first formed portions of the gaseous anode products, or can be largely eliminated by evacuation before the operation is started. Usually, it will be preferred to sweep the system with an inert gas such as nitrogen, helium,  $\text{CF}_4$ , fluorine, and the like, before the operation of the cell is started, preferably before the electrolyte is charged to the cell. The health hazards of fluorine are well known and all appropriate precautions should be taken.

In order to more clearly illustrate this invention, preferred modes of practicing it, and the advantageous results to be obtained thereby, the following examples are given in tabular form in Table I. In these examples, the cell 30 corresponded to that shown in FIGS. 1 and 2 of the drawing, and the various columns of Table I show the anode materials, the temperatures, the current densities, the volts, the times for which the cell was operated, and the results obtained as indicated by the current efficiencies. 35 Boron trifluoride was removed from the off-gas by passing through solid sodium fluoride at  $200^{\circ}$  C. to  $500^{\circ}$  C. Fluorine production was determined by passing the off-gas, freed of boron trifluoride, through a sodium iodide solution and titrating the iodine formed with standardized sodium thiosulfate solution. Sodium, in the sodium-lead alloy, was detected by carefully treating the alloy with water.

Table I

| Example No. | Anode Material                                       | Anode Area (dm. <sup>2</sup> ) | Temp., °C. | Current Density, amp./dm. <sup>2</sup> | Volts | Time, Min. | Current Efficiency, percent |
|-------------|------------------------------------------------------|--------------------------------|------------|----------------------------------------|-------|------------|-----------------------------|
| 1           | Silicon carbide                                      | 0.0126                         | 450        | 2.2                                    | 2.2   | 20         | 58                          |
| 2           | do                                                   | 0.0126                         | 480        | 4.0                                    | 2.2   | 30         | 58                          |
| 3           | Graphite                                             | 0.02                           | 440        | 5.0                                    | 2.2   | 120        | 25                          |
| 4           | do                                                   | 0.02                           | 445        | 5.0                                    | 18.6  | 26         | 25                          |
| 5           | do                                                   | 0.0064                         | 430        | 23.3                                   | 2.2   | 15         | 10.8                        |
| 6           | do                                                   | 0.0064                         | 430        | 15-23.3                                | 2.2   | 15         | 14.7                        |
| 7           | do                                                   | 0.0065                         | 450        | 4.5                                    | 2.2   | 11         | 72.5                        |
| 8           | do                                                   | 0.0065                         | 450        | 4.65                                   | 2.2   | 10         | 92.0                        |
| 9           | do                                                   | 0.10                           | 440        | 2.4                                    | 2.2   | 15         | 11.3                        |
| 10          | do                                                   | 0.10                           | 440        | 2.6                                    | 2.2   | 15         | 10.7                        |
| 11          | do                                                   | 0.10                           | 440        | 2.2                                    | 2.2   | 16         | 32.0                        |
| 12          | do                                                   | 0.10                           | 440        | 2.2                                    | 2.2   | 15         | 23.5                        |
| 13          | Microcrystalline Carbon                              | 0.06                           | 440        | 15-20                                  | 6.6   | 75         | 49.5                        |
| 14          | Explosively compacted graphite, density = 2.1 g./cc. | 0.20                           | 440        | 10-15                                  | 2-2.3 | 54-67 hr.  | 5-42                        |

of molten electrolyte to form a pool 68 of molten lead which extends above the upper end of pipe 62 and forms the cathode for the further operation of the cell. The current is then resumed. Sodium forms at the molten lead cathode 68 and dissolves therein. Fluorine and boron trifluoride form at the anode 56 and pass from the reactor via port 54. The fluorine and boron trifluoride are separated by passing them through sodium fluoride as previously described in connection with the operation of the cell of FIGS. 1 and 2. Liquid sodium-lead alloy is periodically withdrawn from the cathode pool 68 via pipe 62 and valve 64 and more lead is added via port 50. Sodium fluoroborate is also added periodically via port 50.

The current efficiency indicates the order of efficiency of utilization of electric current in forming fluorine. 65 Variations in observed current efficiencies, under substantially identical conditions, were due to variations in naturally occurring impurities, e.g. moisture, in the starting materials which impurities are removed by the electrolysis, and to incomplete recovery of the fluorine due to mechanical difficulties encountered in the recovery system. The current efficiencies were calculated in this manner; when a current of (a) amperes has passed through the cell for (x) seconds a total of (ax) coulombs of electricity has passed through the cell. According to Faraday's law, the formation of one equivalent of

fluorine (i.e. 19 g.) requires one faraday of electricity and one faraday is 96,500 coulombs. Hence, if after time ( $x$ ), it is found that ( $g$ ) equivalents of fluorine have been formed, then 96,500 ( $g$ ) coulombs of current were consumed in the formation of this amount of fluorine. At the same time, a total of ( $ax$ ) coulombs passed through the cell. The current efficiency is then

$$\frac{96500(g)(100)}{(ax)}$$

Taking Example 1, where the current efficiency was 58%, the time was 20 min. = 1200 sec.; the current was 2.2 amps./dm.<sup>2</sup>; the current flow was therefore  $2.2 \times 1200 = 2640$  coulombs/dm.<sup>2</sup>. Hence

$$\frac{96500(g)}{2640} \times 100 = 58$$

or

$$(g) = \frac{58 \times 2640}{100 \times 96500} = 1.586 \times 10^{-2}$$

equivalents of fluorine/dm.<sup>2</sup> or 301.3 milligrams of fluorine/dm.<sup>2</sup> or about 15.07 milligrams of fluorine per minute per dm.<sup>2</sup>.

It will be understood that the foregoing examples have been given for illustrative purposes solely and that this invention is not limited to the specific embodiments described therein. Also, the types and structure of the cell may be widely varied in the manner well known to those skilled in the art in the electrolysis of inorganic fluorine compounds. The materials employed, the temperatures, current densities, volts and the like may be varied within the limits set forth in the general description without departing from the spirit or scope of this invention.

From the foregoing description, it will be apparent that this invention provides a new and improved process for the electrolytic production of fluorine which also produces a valuable cathode product and boron trifluoride as an anode product, which boron trifluoride is readily separated from the elemental fluorine and readily reconverted to sodium fluoroborate which can be recycled to the process, whereby loss of materials as undesired by-products is avoided. The process is simple and readily carried out and results in material economic advantages. Therefore, it will be apparent that this invention constitutes a valuable advance in and contribution to the art.

The embodiments of the invention in which an exclusive property or privilege is claimed are defined as follows:

1. The process for preparing elemental fluorine and a sodium-lead alloy simultaneously which comprises electrolyzing an electrolyte consisting essentially of molten anhydrous sodium fluoroborate in an inert atmosphere at a temperature of from 385° C. to 500° C. in an electrolytic cell having an anode composed of a member of the group consisting of graphite, microcrystalline carbon, and silicon carbide, and a cathode consisting essentially of molten lead at substantially the same temperature as the electrolyte, employing an electric current of from 2 to about 25 volts to provide a current density of from 2 to 50 amps./dm.<sup>2</sup> of anode surface area, recovering a sodium-lead alloy as the cathode product and a gaseous mixture of elemental fluorine and boron trifluoride as the anode product, and separating the elemental fluorine from the boron trifluoride.

2. The process for preparing elemental fluorine and a sodium-lead alloy simultaneously which comprises electrolyzing an electrolyte consisting essentially of molten anhydrous sodium fluoroborate in an inert atmosphere at a temperature of from 385° C. to 500° C. in an electrolytic cell having an anode composed of a member of the group consisting of graphite, microcrystalline carbon, and silicon carbide, and a cathode consisting essentially of molten lead at substantially the same temperature as the

electrolyte, employing an electric current of from 2 to about 7 volts to provide a current density of from 2 to about 20 amps./dm.<sup>2</sup> of anode surface area, recovering a sodium-lead alloy as the cathode product and a gaseous mixture of elemental fluorine and boron trifluoride as the anode product, and separating the elemental fluorine from the boron trifluoride.

3. The process for preparing elemental fluorine and a sodium-lead alloy simultaneously which comprises electrolyzing an electrolyte consisting essentially of molten anhydrous sodium fluoroborate in an inert atmosphere at a temperature of from about 440° C. to about 480° C. in an electrolytic cell having an anode composed of a member of the group consisting of graphite, microcrystalline carbon, and silicon carbide, and a cathode consisting essentially of molten lead at substantially the same temperature as the electrolyte, employing an electric current of from 2 to about 7 volts to provide a current density of from 2 to 20 amps./dm.<sup>2</sup> of anode surface area, recovering a sodium-lead alloy as the cathode product and a gaseous mixture of elemental fluorine and boron trifluoride as the anode product, and separating the elemental fluorine from the boron trifluoride.

4. The process for preparing elemental fluorine and a sodium-lead alloy simultaneously which comprises electrolyzing an electrolyte consisting essentially of molten anhydrous sodium fluoroborate in an inert atmosphere at a temperature of from about 440° C. to about 480° C. in an electrolytic cell having an anode composed of a member of the group consisting of graphite, microcrystalline carbon, and silicon carbide, and a cathode consisting of molten lead at substantially the same temperature as the electrolyte, employing an electric current of from 2 to 3 volts to provide a current density of from 2 to about 4.7 amps./dm.<sup>2</sup> of anode surface area, recovering a sodium-lead alloy as the cathode product and a gaseous mixture of elemental fluorine and boron trifluoride as the anode product, and separating the elemental fluorine from the boron trifluoride.

5. The process for preparing elemental fluorine and a sodium-lead alloy simultaneously which comprises electrolyzing an electrolyte consisting essentially of molten anhydrous sodium fluoroborate in an inert atmosphere at a temperature of from 385° C. to 500° C. in an electrolytic cell having an anode composed of graphite and a cathode consisting essentially of molten lead at substantially the same temperature as the electrolyte, employing an electric current of from 2 to about 25 volts to provide a current density of from 2 to 50 amps./dm.<sup>2</sup> of anode surface area, recovering a sodium-lead alloy as the cathode product and a gaseous mixture of elemental fluorine and boron trifluoride as the anode product, and separating the elemental fluorine from the boron trifluoride.

6. The process for preparing elemental fluorine and a sodium-lead alloy simultaneously which comprises electrolyzing an electrolyte consisting essentially of molten anhydrous sodium fluoroborate in an inert atmosphere at a temperature of from 385° C. to 500° C. in an electrolytic cell having an anode composed of explosively compacted graphite and a cathode consisting essentially of molten lead at substantially the same temperature as the electrolyte, employing an electric current of from 2 to about 25 volts to provide a current density of from 2 to 50 amps./dm.<sup>2</sup> of anode surface area, recovering a sodium-lead alloy as the cathode product and a gaseous mixture of elemental fluorine and boron trifluoride as the anode product, and separating the elemental fluorine from the boron trifluoride.

7. The process for preparing elemental fluorine and a sodium-lead alloy simultaneously which comprises electrolyzing an electrolyte consisting essentially of molten anhydrous sodium fluoroborate in an inert atmosphere at a temperature of from about 440° C. to about 480° C. in an electrolytic cell having an anode composed of

explosively compacted graphite and a cathode consisting essentially of molten lead at substantially the same temperature as the electrolyte, employing an electric current of between 2 and 3 volts to provide a current density of from 2 to about 20 amps./dm.<sup>2</sup> of anode surface area, recovering a sodium-lead alloy as the cathode product and a gaseous mixture of elemental fluorine and boron trifluoride as the anode product, and separating the elemental fluorine from the boron trifluoride.

8. The process for preparing elemental fluorine and a sodium-lead alloy simultaneously which comprises electrolyzing an electrolyte consisting essentially of molten anhydrous sodium fluoroborate in an inert atmosphere at a temperature of from 385° C. to 500° C. in an electrolytic cell having an anode composed of microcrystalline carbon and a cathode consisting essentially of molten lead at substantially the same temperature as the electrolyte, employing an electric current of from 2 to about 25 volts to provide a current density of from 2 to 50 amps./dm.<sup>2</sup> of anode surface area, recovering a sodium-lead alloy as the cathode product and a gaseous mixture of elemental fluorine and boron trifluoride as the anode product, and separating the elemental fluorine from the boron trifluoride.

9. The process for preparing elemental fluorine and a sodium-lead alloy simultaneously which comprises electrolyzing an electrolyte consisting essentially of molten anhydrous sodium fluoroborate in an inert atmosphere at a temperature of from 385° C. to 500° C. in an electrolytic cell having an anode composed of a member of the group consisting of graphite, microcrystalline carbon, and silicon carbide, and a cathode consisting essentially of molten lead at substantially the same temperature as the electrolyte, employing an electric current of from 2 to about 25 volts to provide a current density of from 2 to 50 amps./dm.<sup>2</sup> of anode surface area, recovering a sodium-lead alloy as the cathode product and a gaseous mixture of elemental fluorine and boron trifluoride as

the anode product, separating the elemental fluorine from the boron trifluoride by passing the gaseous mixture through sodium fluoride at a temperature of from about 200° C. to about 500° C. whereby the boron trifluoride reacts with the sodium fluoride to reform sodium fluoroborate, and recycling the reformed sodium fluoroborate to the electrolytic cell.

10. The process for preparing elemental fluorine and a sodium-lead alloy simultaneously which comprises electrolyzing an electrolyte consisting essentially of molten anhydrous sodium fluoroborate in an inert atmosphere at a temperature of from about 440° C. to about 480° C. in an electrolytic cell having an anode composed of graphite and a cathode consisting essentially of molten lead at substantially the same temperature as the electrolyte, employing an electric current of between 2 and 3 volts to provide a current density of from 2 to about 20 amps./dm.<sup>2</sup> of anode surface area, recovering a sodium-lead alloy as the cathode product and a gaseous mixture of elemental fluorine and boron trifluoride as the anode product, separating the elemental fluorine from the boron trifluoride by passing the gaseous mixture through sodium fluoride at a temperature of from about 200° C. to about 500° C. whereby the boron trifluoride reacts with the sodium fluoride to reform sodium fluoroborate, and recycling the reformed sodium fluoroborate to the electrolytic cell.

#### References Cited by the Examiner

##### UNITED STATES PATENTS

|           |       |                 |       |        |
|-----------|-------|-----------------|-------|--------|
| 2,848,396 | 8/58  | Murphy et al.   | ----- | 204—60 |
| 2,918,417 | 12/59 | Cooper et al.   | ----- | 204—60 |
| 2,940,911 | 6/60  | Uchiyama et al. | ----- | 204—60 |
| 3,017,336 | 1/62  | Olsowski        | ----- | 204—64 |

WINSTON A. DOUGLAS, *Primary Examiner.*

JOHN R. SPECK, JOHN H. MACK, *Examiners.*